# EUROPEAN PATENT SPECIFICATION

(11) **EP 1 171 304 B1**
(45) Date of publication and mention of the grant of the patent: **10.09.2003**
(21) Application number: 00917187.7
(22) Date of filing: 06.04.2000
(51) Int. Cl.: B41C 1/18, B41N 7/00

(54) **IMPROVED GRAVURE PRINTING ROLLERS**
TIEFDRUCKZYLINDER
ROULEAU DE PRESSE A HELIOGRAVURE AMELIORE

(30) Priority: 07.04.1999 GB 9907784; 11.06.1999 GB 9913643
(43) Date of publication of application: 16.01.2002
(73) Proprietor: Hyperlast Limited, High Peak, Derbyshire SK22 1BR (GB)
(72) Inventor: MOSS, Robert Malcolm, Glossop, Derbyshire SK13 6LH (GB); CAMPION, John William, NR Preston, Lancashire PR3 0AN (GB); ARMFIELD, Sidney Robert, Urmson, Manchester M41 6ER (GB)
(74) Representative: Wilson Gunn M'Caw
(86) International application number: GB0001301
(87) International publication number: WO00059727

(56) References cited:
- EP-A- 0 038 385
- EP-A- 0 344 332
- EP-A- 0 364 653
- EP-A- 0 384 104
- WO-A-99/32302
- M. ALGER: "Polymer Science Dictionary" , CHAPMAN&HALL , LONDON SE1 8HN UK XP002143017 page 551 -page 552

## Description

This invention relates to improvements in gravure printing rollers.

At present, gravure printing rollers are usually machined to the required size from stainless steel. Stainless steel rollers are however extremely heavy which is a major disadvantage, both from the point of view of transportation, and also in changing rollers in a printing machine.

Accordingly, it has been long considered desirable to be able to use rollers of a lower weight material, such as a composite including a relatively low density synthetic material which retains a durable printing face such as chrome treated copper, yet is light to ease shipping and handling.

It has been found that standard foam material is unsuitable for this purpose as the moulded foam core requires sealing with a filler to close the pores to enable a pore and void-free copper coating to be deposited and subsequently chrome treated as a print face. Even if a skinning foam is used to produce a roller shell, the great diversity of gravure roller diameters requires that a machining operation is used to reduce the roller shell diameter to the designed value, which exposes foam pores which require filling.

Further, the equipment required to produce a foam core is complicated because it is necessary to use clamping force to hold in the foam during the moulding cycle.

There have been a number of proposals for lightweight printing rollers of various kinds, for example FULLER, WO 99/32302 proposes a printing roller comprising a body of low density hard foam, and a surface layer comprising a non-foamed polyurethane including 15 - 70% filler such as chalk. ROSSINI, EP-A-384,104 describes a roll comprising a stiff inner core, having a shell of rigid expanded polyurethane, which is smoothed and electroplated with a layer of copper. BARDIN, EP-A-0038385 forms a roll by moulding a body of plastics material, machines the roll to size and plates the machined surface with copper.

TOKYO KOKAI, EP-A-0364,653 describes a roller which comprises a substrate which includes hollow microspheres. The printing surface is produced by grinding and rupturing the microspheres to provide a roughened surface to aid ink retention. Similarly, KINYOSHI, EP-A-0,344,332 describes a roller with mineral particles embedded in a surface layer. The surface provides a surface which pits and projects at the particle scale, which again is said to aid ink retention.

The invention provides a gravure roller comprising a lightweight shell made from a syntatic moulding composition comprising a polyurethane matrix containing hollow microspheres, characterised in that the shell (15) has a non-porous machine surface with a printing face of chrome treated copper deposited on the surface.

A syntactic moulding composition is defined for the purpose of this specification as being a synthetic matrix including preformed beads providing discrete bubbles. This composition is capable of providing a uniform cellular construction of homogenous and consistent density which can be machined without leaving a porous or void containing surface.

The syntactic moulding composition preferably comprises a polyurethane composition formed into preformed plastics beads each comprising an individual shell surrounding an interior void and bonded by a polyurethane composition. The beads may be in the size range of 20 to 100 µm (microns) (weight average diameter) and may alternatively comprise other polymers, glass, or ceramic beads.

The invention also provides a method of manufacturing gravure roller, comprising moulding a roller shell from a syntatic moulding composition comprising a polyurethane matrix containing hollow microspheres, machining the peripheral surface of said roller shell to produce a non-porous machined surface and depositing a layer of chrome treated copper on the surface to provide a printing face.

The shell may advantageously be mechanically reinforced, to prevent flexure of the roller, by means of a rigid tubular core upon which the shell is moulded. The core may be for example of glass reinforced plastics, or a concrete composition.

The polyurethane used in the moulding composition can be manufactured from a range of ingredients. For example, polyether or polyester polyols may be used, with any of the common isocyanates; including methylene diphenyl diisocyanate; toluene diisocyanate; naphthalene diisocyanate; tetramethyl xylidene diisocyanate; isophorone diisocyanate; phenylene diisocyanate; cyclohexyl diisocyanate; xylidene diisocyanate; hexamethylene diisocyanate; as well as biuret, allophanate and prepolymeric adducts of these. Diol, triol, polyol or polyamine crosslinkers may be used, with an amine or metal catalyst which is preferably of a type which negates blowing reaction in the moulding step following bead expansion.

The isocyanate component may be pre-polymerised and contain the expansion agent so that the isocyanate component is a low density liquid whilst the polyol is a standard polyol.

A suitable composition may be as follow:-

| Polyol component:- (by weight ) | |
|---|---|
| Castor Oil - | 46.8 |
| Polyether hexol - | 46.8 |
| Antifoam - | 0.19 |
| Dessicant - | 2.4 |
| Catalysts - | 0.25 |
| Expancel 551DE - | 3.59 |
| Isocyanate:- | |
| Polymeric methylene diphenyl diisocyanate (MDI) - | 100% |
| Mix ratio: | 60 parts polyol to 50 parts of isocyanate |
| Gel time at 25°C - | 10 to 15 minutes |
| Hardness - | 70 shore D |
| Density - | 0.72 |
| Viscosity polyol - | 400 poise at 25°C |

The moulding is carried out at 60°C in a low pressure two component polyurethane dispenser-2KM machine.
In accordance with this invention, the surface of the syntactic moulding polyurethane composition is, after machining, preferably treated with a conductive coating to provide a host surface for the copper plating.

This has been found to be necessary as the preferred syntactic polyurethane composition keys poorly to the cooper plating so that there is low adhesion between the machined roller surface and the cooper layer.

The conductive coating is preferably an organic solvent based composition containing one or more conductive agents. The latter may comprise additions of conductive materials such as finely divided metals, or additives which adjust the ionic state of the coating to render it conductive.

The rollers may be manufactured entirely from the syntactic moulding composition ,whilst in other possible embodiments, the roller shells are fitted with steel or aluminum end plates and/or shafts or trunnions.

The rollers according to the invention may be used not only for gravure printing, but also for flexo printing.

The invention will now be further described by way of example, with reference to the accompanying drawings, wherein:-
- Figure 1: is a simplified cross-sectional view of a gravure roller according to the invention;
- Figure 2: is an enlarged sectional view of part of the roller shell;
- Figure 3: is a much enlarged sectional view showing the results obtained by working a conventional urethane foam; and
- Figure 4: is a similar enlarged sectional view of the structure of a surface produced by working a syntactic foam on a roller according to the invention.

In Figure 1, a gravure roller 1 is shown which comprises a roller body or shell 15. In accordance with the invention the roller shell body 15 is made by moulding a syntactic polyurethane foam, which is then machined to achieve the desired diameter and produce a substantially non-porous and void-free outer surface 16, on which a layer of copper 17 is deposited after treatment with a conductive coating which provides adhesion for the copper, and then treated with chrome and processed as required to act as a gravure printing roller. The roller also includes a tubular core 12, which acts as a support and reinforcing member to prevent or minimise flexure of the roller, with end caps 13, 14 formed with trunnions 11so that the roller 1 can be mounted in a machine. The core is of a suitably strong material, such as glass reinforced plastics, or a concrete composition, particularly a resin bonded concrete.

The conductive composition is an organic based coating including a conductive agent such as powdered metal or ionic adjusting additives.

A portion of the roller shell 15 with the copper layer 17 thereon is shown in Figure 2.

Figure 4 shows, much magnified, the surface 16 of the roller shell 15, wherein the bonded beads or bubbles 18 of polyurethane or other plastics foam are shown in a polyurethane matrix 19 and providing a substantially non-porous surface 16 free of major voids and with only micros-pits caused by the opening or removal of individual beads 18. The beads may alternatively be of glass or ceramic material.

By contrast, Figure 3 shows a machined surface 116 of a layer 115 of a normal open-celled foam which has, for example, been poured into the mould as liquid and allowed to cure and foam simultaneously in the mould. As shown, the foam, after planarising , has major voids 117 and pores 118 which, by linking of adjacent foam cell, often penetrate well in to the foam body so that the surface 116 is by no means non-porous or free voids.

The roller shell 15 is made by moulding a syntactic polyurethane foam. This is then machined to the required size, a coat of a special paint applied over the surface, copper deposited and the shell is then assembled into the roller structure for subsequent chromium plating, etching and use in printing.

The roller may weigh about 5 to 7 kg instead of the weight of 100 kg when steel is used for the roller shell.

The roller can be refurbished by recoating with copper and rechromium plating and etching. The relatively light weight ensures that transportation and handling, including mounting and dismounting the roller is easy and imposes no handling problems. A roller formerly requiring use of a 7.5 tonne truck for delivery of a set of rollers can now be delivered using a light weight van.

Because of the reduced weight of the shell, the other parts of the roller, including the end plates, shaft and trunnions, can be made of reduced weight materials, e. g. lightweight metals such as aluminium alloys, or synthetic materials such as suitable rigid plastic materials including forming all or part of the roller from the syntactic foam material.

A preferred syntactic foam composition used in manufacture of the shell is preferably as set out above.

Alternatively, moulding may be carried out with a polyisocyanate composition, using a prepolymer with a polyester or polyether polyol, a friability modifier and an isocyanate catalyst such as DABCO TMR5.

Other urethane derivatives can be polyoxazolidone produced by means of epoxy/isocyanate addition compositions.

As an alternative to polyurethane, the syntactic material can be based on other polymers such as unsaturated polyesters, vinyl esters or polyacrylic systems such as Modar (Trade Mark of ICI) can be used.

## Claims

1. A gravure roller comprising a lightweight shell (15) made from a syntactic moulding composition comprising a polyurethane matrix containing hollow microspheres, (18) **characterised in that** the shell (15) has a non-porous machined surface (16) with a printing face of chrome treated copper deposited on the surface (16).

2. A gravure roller according to claim 1, **characterised in that** a conductive coating is deposited on the surface (16) before depositing the chrome treated copper thereon.

3. A gravure roller according to claim 1 wherein said hollow microspheres comprise hollow beads, (18) with a shell of polyurethane, glass or ceramic material surrounding an interior void.

4. A gravure roller according to claim 2 wherein the conductive coating comprises an organic solvent based composition containing one or more electrically conductive agents.

5. A gravure roller according to claim 4, wherein the conductive agent or agents comprise an additive of one or more electrically conductive finely divided metals.

6. A gravure roller according to claim 4, wherein the conductive agent comprises an additive which adjusts the ionic state of the coating to render it electrically conductive.

7. A gravure roller according to claim 3 wherein the beads (18) have a size range of from 20 to 100 µm (microns).

8. A gravure roller according to any preceding claim wherein the shell (15) is formed on a reinforcing core.

9. A method of manufacturing a gravure roller, comprising moulding a roller shell (15) from a syntatic moulding composition comprising a polyurethane matrix containing hollow microspheres (18), machining the peripheral surface of said roller shell (15) to produce a non-porous machined surface (16) and depositing a layer of chrome treated copper on the surface (16) to provide a printing face (17).

10. A method according to claim 9 comprising coating the machined surface (16) with a conductive coating before depositing the layer of chrome treated copper.

## Patentansprüche

1. Druckzylinder, der eine leichte Schale (15) aus einer syntaktischen Gießmasse mit einer Polyurethanmatrize umfasst, welche hohle Mikrokugeln (18) enthält, **dadurch gekennzeichnet, dass** die Schale (15) eine porenlose, maschinell bearbeitete Oberfläche (16) mit einer Druckfläche aus verchromtem Kupfer aufweist, das auf der Oberfläche (16) aufgebracht ist.

2. Druckzylinder nach Anspruch 1, **dadurch gekennzeichnet, dass** auf der Oberfläche (16) eine leitfähige Schicht aufgebracht wird, bevor auf dieser die verchromte Kupferschicht aufgebracht wird.

3. Druckzylinder nach Anspruch 1, wobei die hohlen Mikrokugeln hohle Perlen (18) umfassen, mit einer Schale aus Polyurethan-, Glas- oder Keramikmaterial bestehen, welche einen leeren Innenraum umschließen.

4. Druckzylinder nach Anspruch 2, wobei die leitfähige Beschichtung eine Zusammensetzung auf der Basis eines organischen Lösungsmittels umfasst, welche ein oder mehrere elektrisch leitfähige Materialien enthält.

5. Druckzylinder nach Anspruch 4, wobei das leitfähige Material oder die leitfähigen Materialien ein Additiv umfasst, das ein oder mehrere elektrisch leitfähige, fein verteilte Metalle enthält.

6. Druckzylinder nach Anspruch 4, wobei das leitfähige Material ein Additiv umfasst, welches den lonenzustand der Beschichtung darauf einstellt, sie elektrisch leitfähig zu machen.

7. Druckzylinder nach Anspruch 3, bei welchem die Perlen (18) einen Größenbereich von 20 bis 100 µm (Mikron) haben.

8. Druckzylinder nach einem der vorhergehenden Ansprüche, bei welchem die Schale (15) auf einem Verstärkungskern ausgebildet ist.

9. Verfahren zur Herstellung eines Druckzylinders, das die Folgendes umfasst:
Gießen einer Zylinderschale (15) aus einer syntaktischen Gießmasse, die eine Polyurethanmatrize umfasst, welche hohle Mikrokugeln (18) enthält;
maschinelle Bearbeitung der Umfangsoberfläche der Zylinderschale (15), um eine porenlose, maschinell bearbeitete Oberfläche (16) zu erzeugen und
Aufbringen einer Schicht aus verchromtem Kupfer auf die Oberfläche (16), um eine Druckfläche (17) bereitzustellen.

10. Verfahren nach Anspruch 9, umfassend die Beschichtung der maschinell bearbeiteten Oberfläche (16) mit einer leitfähigen Beschichtung vor dem Aufbringen der Schicht aus verchromtem Kupfer.

## Revendications

1. Rouleau de gravure comprenant une coque légère (15) formée d'une composition de moulage syntactique comprenant une matrice de polyuréthane contenant des microsphères creuses (18), **caractérisé en ce que** la coque (15) possède une surface usinée non poreuse (16) possédant une face d'impression en cuivre traitée au chrome, déposée sur la surface (16).

2. Rouleau de gravure selon la revendication 1, **caractérisé en ce qu'**un revêtement conducteur est déposé sur la surface (16) avant le dépôt, sur cette surface, du cuivre traité au chrome.

3. Rouleau de gravure selon la revendication 1, dans lequel lesdites microsphères creuses comprennent des billes creuses (18) possédant une coque en polyuréthane, en verre ou en matériau céramique entourant un vide intérieur.

4. Rouleau de gravure selon la revendication 2, dans lequel le revêtement conducteur comprend une composition basée sur un solvant organique contenant un ou plusieurs agents électriquement conducteurs.

5. Rouleau de gravure selon la revendication 4, dans lequel le ou les agents conducteurs comprennent un additif d'un ou de plusieurs métaux électriquement conducteurs, finement divisés.

6. Rouleau de gravure selon la revendication 4, dans lequel l'agent conducteur comprend un additif qui ajuste l'état ionique du revêtement pour le rendre électriquement conducteur.

7. Rouleau de gravure selon la revendication 3, dans lequel les billes (18) possèdent une gamme de tailles allant de 20 à 100 µm (micromètres)

8. Rouleau de gravure selon l'une quelconque des revendications précédentes, dans lequel la coque (15) est formée sur un noyau de renfort.

9. Procédé pour fabriquer un rouleau de gravure, consistant à mouler une coque de rouleau (15) à partir d'une composition de moulage syntactique comprenant une matrice de polyuréthane contenant des microsphères creuses (18), à usiner la surface périphérique de ladite coque (15) du rouleau pour produire une surface usinée non poreuse (16) et déposer une couche de cuivre traité au chrome sur la surface (16) pour former une face d'impression (17).

10. Procédé selon la revendication 9, consistant à recouvrir la surface usinée (16) par un revêtement conducteur avant de déposer la couche de cuivre traitée au chrome.
